

J. A. LOCKHART.

WALL BOARD AND PLASTER COMPOSITION ADAPTED THERETO.

APPLICATION FILED APR. 8, 1921.

1,423,569.

Patented July 25, 1922.

Fig 1



Fig 2



Fig 3



JAMES A. LOCKHART  
INVENTOR

BY *Johns Power*  
ATTORNEY

# UNITED STATES PATENT OFFICE.

JAMES A. LOCKHART, OF BUFFALO, NEW YORK, ASSIGNOR TO PITHO PLASTIC BOARD COMPANY, INC., OF BUFFALO, NEW YORK, A CORPORATION OF NEW YORK.

## WALL BOARD AND PLASTER COMPOSITION ADAPTED THERETO.

1,423,569.

Specification of Letters Patent. Patented July 25, 1922.

Application filed April 8, 1921. Serial No. 459,737.

*To all whom it may concern:*

Be it known that I, JAMES A. LOCKHART, a citizen of the United States, residing at Buffalo, in the county of Erie and State of 5 New York, have invented certain new and useful Improvements in Wall Board and Plaster Compositions Adapted Thereto, of which the following is a specification.

This invention relates to improvements in 10 wall board and plastic compositions adapted thereto.

The objects of the invention are to provide wall board which shall be very light in weight, which shall be without brittleness 15 and which will not crack consequent to nailing, which shall be waterproof and fireproof, whose body shall be sufficiently porous to produce good suction effects and whose surface shall be sufficiently rough to produce 20 good keying effects in connection with the application of outside finishing material, such as Keene or Portland cement or stucco, and which shall be exceedingly cheap to manufacture.

25 In the accompanying drawing;

Figure 1 is an elevation of the wall board in accordance with the invention, showing more particularly the rough surface thereof to which the finishing material is applied.

30 Figure 2 is a sectional view of the same, and

Figure 3 is a view showing the shredded wood fibres which constitute an essential ingredient of the wall board.

35 The ingredients of the composition are plaster of Paris, lime (stone or refined) and shredded wood fibres.

While the proportions of the composition are not absolute I have found that the best 40 results are obtained by providing about three parts, by weight, of plaster of Paris for one part of lime, and by providing the shredded wood fibres in a quantity slightly less, by weight, than the plaster of Paris.

45 The shredded wood fibres are not to be confounded with excelsior saw dust, paper pulp or any merely generically required fibrous filler. These shredded wood fibres have a definite and characteristic form and 50 a definite proportional relation to the finished wall board and by virtue of such form and relation advantageous results are obtained in course of manufacture and advantageous and novel qualities are imparted to the finished wall board.

By the term "shredded wood fibres" as used herewith and in the claims I refer to wood fibres of peculiar formation, that is to say fibres which are from three-quarters of an inch to one and one-quarter of an inch 60 in length, more or less, and are quite coarse, somewhat irregular in their form and for the most part of what might be called compound formation, that is to say several of the fibres running in the same general direction will be somewhat loosely united as a cluster. As far as practical the fibres are illustrated in Fig. 3. They are, of course, light and flexible, although having sufficient coarseness and stiffness. 70

The ingredients are thoroughly mixed together, after which the composition is compressed and formed into wall board in any suitable or known manner, one surface of the board, however, being left rough or unfinished, as shown in Figures 1 and 2, and the other surface being preferably smooth. The rough surface cooperates with outside finishing material such as cement or stucco and the smooth surface cooperates with inside finishing material such as paint, calcimine or wall paper. 75

For most industrial purposes the finished wall board should be about a quarter of an inch thick, the shredded wood fibres 80 being several times greater in length than the thickness of the board. These fibres not only extend throughout the entire mass, functioning most effectually as a reinforcement, but also will be exposed along the 85 surface of the board and will produce the desired and requisite roughness of the surface to which the finishing material is to be applied. As exposed along such roughened surface the shredded wood fibres will extend in all directions in the general plane of such surface and will also extend at various angles to such plane. Thus the roughened surface is characterized by closely associated ridges, projections and indentations of irregular form, proportion and extent by virtue of which good keying effects are produced. 95

The fibres, by virtue of their body, i. e., coarseness and "clustering," relative stiffness and irregularity of outline, while serving most effectually as a re-inforcement for the plastic ingredients, will also prevent such ingredients from becoming too intimately packed together under pressure. 100 110

This preserves a certain porosity throughout the mass which is not incompatible with good waterproof qualities but which has the advantages, first of enabling the board to 5 dry very quickly in course of manufacture, and second, of providing for efficient suction effects when the finishing material, Keene or Portland cement or stucco is applied. These suction effects in connection 10 with the keying effects of the roughened surface insure a most secure application of the finishing material.

The shredded wood fibres in addition to the advantages specified also eliminate any 15 quality of brittleness or friability, and insure that the wall board will not crack under nailing.

In addition to the material specified a small quantity of sand may be added to give 20 a body but while this is preferred it is not at all necessary.

Having fully described my invention, I claim:

1. Plaster composition for wall board 25 comprising plaster of Paris, lime and shredded wood fibres.
2. Plaster composition for wall board

comprising plaster of Paris, lime and shredded wood fibres in the proportions, by weight, of three parts plaster of Paris to 30 one part of lime and the shredded wood fibres in slightly less quantity than the plaster of Paris.

3. Wall board composed of plastic material and shredded wood fibres incorporated 35 therein, the fibres being several times greater in length than the thickness of the board and producing a roughened surface to which finishing material may be applied.

4. Wall board composed of a mixture of 40 plaster of Paris and lime and shredded wood fibres incorporated therein, the fibres being several times greater in length than the thickness of the board.

5. Wall board composed of a mixture of 45 plaster of Paris and lime and shredded wood fibres incorporated therein, the fibres being several times greater in length than the thickness of the board and producing a roughened surface to which finishing ma- 50 terial may be applied.

In testimony whereof I affix my signature.

JAMES A. LOCKHART.